

## UNITED STATES PATENT OFFICE

2,042,347

## CHEMICAL CLEANING PROCESS

Franklin H. Mackenzie, Bywood, Pa., assignor  
to American Chemical Paint Company,  
Ambler, Pa.

No Drawing. Application March 13, 1935,  
Serial No. 10,937

2 Claims. (Cl. 87—5)

The invention relates to a chemical cleaning process wherein chemical cleaners are used for the cleaning of various materials such as metal, fabrics, cotton, wool or silk in the raw state, 5 bottles, barrels, etc., and the invention is applicable in connection with any industrial process where the cleaning solutions are used in tanks or cleaning equipment. The present application is a continuation in part of my application Serial 10 No. 557,717, filed August 17, 1931.

Such chemical cleaners in general include two principal active agents, namely, an alkali agent and an emulsifying compound. The alkali agent is composed of salts of the alkali metals, such as 15 sodium or potassium phosphates, silicates, carbonates, hydroxides, borates, etc., mixed to have the proper buffering and inhibiting properties together with the cleaning ability for the work to be done.

20 The emulsifying compound is composed of substances that will reduce the inter-facial tension. There are a great number and variety of these materials, only a few of which will be mentioned here, i. e., soaps, fatty acids, glues, proteins, sulfonated oils, rosin, finely divided and cellular inert materials, etc.

These two factors, namely, the alkali and the emulsifier, which together go to make up the ordinary alkali chemical cleaning compound, give 30 rise to two distinct detergent properties or functions in the chemical cleaner. Thus the action of the alkalies is principally chemical in its nature, tending to soften the water, saponify vegetable and animal oils, neutralize acids and conduct electricity. The action of the emulsifier, on the other hand, is the reduction of inter-facial tension, colloidal suspension or adsorption and results in wetting out the dirt and oil, deflocculating and suspending the same; or the adsorption 35 of oil by finely divided inert materials. This action is mainly mechanical and depends upon agitation for its proper functioning. Since the two factors are distinct in their nature, it is desirable that each should be separately regulatable 40 according to the requirements of any particular cleaning operation.

It is common practice for manufacturers to make up ready-mixed cleaners which are combinations of an emulsifying agent and an alkali 50 mixture. Certain compounds are found, in practice, to be far superior to others for certain classes of work, and it is accordingly necessary to provide an almost infinite number of compounds differing from each other in the relative properties of the two principal factors.

Such ready-mixed compounds possess the disadvantage that it is impossible to accurately control the emulsification properties of the cleaning solution employed, because in most instances soaps are formed by the action of the chemicals 5 on the oils removed from the article being cleaned, and thus additions of the ready-mixed cleaner containing both the alkali mixture and the emulsifier must necessarily increase the emulsifying power of the solution, whether such addition of emulsifier is necessary or not, thus resulting in a waste of the emulsifier.

The use of too great a proportion of the emulsifier will, moreover, cause too much oil and inert matter to be held in the solution by the emulsifier. The solution thus tends to become progressively more and more viscous, and even though the alkalinity may be raised to a considerable degree, the detergent properties of the cleaner fall off considerably, and after a period 20 of time, the solutions have to be dumped and renewed, owing to the excess of the emulsifier contained therein.

A very unsatisfactory condition will also result if too small an amount of emulsifier is used in the mixture or if the amount of saponifiable material coming into the tank from the work is not sufficient or if it varies in quantity, as the solution will then lack the ability to remove mineral oils and foreign material. The emulsification property in a metal cleaner is very important as practically all steel is slushed at the mill with a mineral oil and picks up inorganic matter or unsaponifiable dirt.

35 A close observation of the detergent properties of alkali cleaners reveals the fact that it is almost an impossibility to keep a cleaning solution working at maximum efficiency with cleaners having the emulsifying agent incorporated in them, as any change in the character of the work will throw the solution out of balance for most efficient cleaning. Also considerable research work is necessary to compound a cleaner correctly even where the work remains constantly the same.

40 According to my invention, the alkali mixture and the emulsifier are furnished separately and a cleaning solution prepared at the place of use by mixing proper quantities of the alkali mixture and of the emulsifier with water.

50 The resultant solution is heated to the desired temperature and the work to be cleaned is treated with the cleaning solution in the usual manner whether it be soaking in a boiling solution, agitating in solutions of various temperatures, 55

spraying the solution on the work, using direct or alternating current from work to the tank or anodes or by a process of dipping work in solution and wringing. During the process of cleaning, the cleaning solution is tested at suitable intervals for both alkalinity and emulsifying power, and the necessary quantities of one or both ingredients are added according to the results of the test.

10 It will be understood that the present invention is not concerned with the particular manner in which the materials undergoing treatment are cleaned, as this varies with circumstances and is also dependent on the character 15 of the materials being cleaned, the invention being applicable to the various commonly known types of cleaning processes enumerated above. Also, the present application is not primarily concerned with the particular manner of testing the cleaning solution for alkalinity or emulsifying power, but for the purpose of illustration the preferred methods of carrying out these individual steps which form a part of the combined process constituting the principal feature of the 20 present application will be described in detail. Special forms of equipment for carrying out these tests for alkalinity and emulsifying power have been designed, which I term testing kits.

25 The testing may be carried out in the following manner:

#### Alkalinity test

The test for the alkali mixture may consist of the titration of a 10 cc. portion of the cleaning 35 solution with an acid solution of known strength using phenolphthalein as an indicator as in chemical analysis. The preferred process, however, is distinctive in that it has been simplified for production use. The normality of the acid is 40 adjusted to a value which will make the calculations involve no more than two digits. The indicator is incorporated in the acid by using an alcohol solution of the indicator instead of distilled water to adjust the normality. The alkali mixtures are numbered according to the amount 45 of material present that is capable of being titrated (with the particular normality acid and indicator described above) in such a manner that the titration of a 10 cc. sample of the cleaner 50 solution multiplied by the number of the material equals ounces per gallon of the cleaner in solution.

In the form of an example, the titration of a 10 cc. portion of the cleaning bath is as follows:

55 Number of cc. of acid used times number of material equals ounces per gallon of cleaner in solution.

Still further simplification is effected in the process as actually carried out, which consists of 60 determining a tank factor for each tank and this, when multiplied by the titration, equals pounds of cleaner per tank. The tank factor is obtained by multiplying the number of gallons in the tank by the number of the material divided by 16 as

65 Number of material used  $\times$  number of gallons in tank

16

Alkali tank factor  $\times$  number of cc. used in titrating 10 cc. sample = number pounds per tank. It is obvious that by this system the operator makes an accurate determination of the cleaner content by a simple titration and an easy multiplication, giving results in terms similar to those used for additions.

75 Also it is obvious that this system could be

applied to all systems of weights and measures.

#### Emulsifier test

The problem of testing for emulsifying power is not to show the amount of the emulsifier as in ordinary analysis (as emulsifiers are constantly coming into the bath in the process of cleaning and it would be necessary to analyze for each type of emulsifier, separate them, and also know their effectiveness to keep the emulsifying power of the bath constant), but to show the effectiveness in such a way that it can be interpreted in terms of a known emulsifier.

The best emulsifier available for the operation is used and for a given concentration in the bath its properties, i. e., inter-facial tension reduction and colloidal suspension, are measured in a unique manner suitable for production conditions. The result in minutes is converted into a factor which when multiplied by the time in future tests will indicate the amount of emulsifier present, not by actual quantity, but by its effectiveness.

It is obvious that any emulsifier may come into the solution, and without knowing its characteristics or concentration, its effectiveness in the bath may be ascertained and the bath adjusted to the proper emulsification value with the original emulsifier.

A suitable device for measuring the emulsifying power of the bath may consist of a tall narrow glass cylinder or bottle having a broad base suitable for supporting it in a vertical position, the bottle being preferably provided with a ground glass stopper. A glass bottle six inches 35 high and one-half inch in diameter has proved satisfactory in actual practice. This bottle is marked with suitably selected graduations designated as "Time", "Oil" and "Sol" (solution). Of these the time graduation is lowest, the sol grad- 40 uation next and the oil graduation uppermost.

The test is conducted in the following manner: The cylinder is filled to the solution level (Sol) marked on the bottle, with a sample of the cleaning bath when first made up. A clear white 45 mineral oil, viscosity 120 to 130 seconds at 100° F. (Saybolt) is added until it reaches a graduation on the bottle marked "Oil" level. For most accurate work, the cylinder is stoppered and immersed in a water bath at 140° F., the bath al- 50 lowed to cool to 130° F., and the cylinder removed. In ordinary commercial operation, the water bath treatment need not be resorted to, as the variation in temperature is usually not sufficient to cause a serious error.

The cylinder is shaken rapidly 25 times and stood vertically on its base. The time is accurately recorded, from the moment the cylinder is placed in a vertical position, until the emulsion level reaches a graduation on the bottle marked "Time". The emulsion level is the level where the cleaning solution meets the emulsion. As the emulsion breaks, the cleaning solution falls to

65

= alkali tank factor.

the bottom, forcing the emulsion higher. The meeting point of the cleaning solution and the emulsion forms a definite line that cannot be 70 mistaken, as the solution is clear and the emulsion opaque.

This time is in direct proportion to the emulsifying power of the bath and also in a direct proportion to the amount of emulsifier used.

75

The time in minutes is divided into the number of fluid ounces of emulsifier used, which gives the emulsification factor for that particular tank,

alkalinity and for emulsification. A lack of either alkali or emulsifier may be determined in this manner, and the bath brought to proper concen-

5      Number fluid ounces of emulsifier used  
Number minutes required for emulsion level to rise to line mark = emulsification tank factor

10     Tests in the future are run in the same manner. The time multiplied by the emulsification tank factor equals number of fluid ounces of emulsifier or its equivalent in emulsifying power in the bath, from which information the proper additions may be made.

15     Time  $\times$  emulsification tank factor = number of fluid ounces of emulsifier in tank or its equivalent in emulsifying power.

20     It is evident from the above method of test that when saponifiable material comes into the bath from the work and is saponified, account is taken of its emulsifying power which reduces the amount of original emulsifier needed to keep the proper concentration of emulsifier. In this manner, the saponifiable material is utilized and excessive amounts of emulsifier are avoided. With 25 my proposed method of control, the chemical cleaner solution may be run almost indefinitely on any type of work, as the emulsification factor may be raised to the point necessary to do the work properly, and the quantity limited so that 30 the emulsifier will not hold oil or foreign matter in suspension too long. The dirt which precipitates may be removed from the bottom of the cleaning tank by hoeing it out or pushing it over toward the drain and allowing it to pass down 35 the drain.

35     Any oil which precipitates may be removed by bringing the level up to the overflow and allowing it to pass over the overflow, or by skimming the oil off with a skimmer. The removal of dirt and excess oil may be performed periodically, generally each morning, after the solution has been allowed to settle overnight, for the oil, and once a week for the dirt.

40     By employing my process, marked economies result which consist of the elimination of frequent dumping, due to solution going out of balance with respect to the emulsifier content and the resultant building up of a heavy dirt and oil load; keeping the bath uniform produces uniform work, thus eliminating rejects and producing a more stable solution for automatic equipment where the work must be cleaned in a definite time; saving in the amount of emulsifier used where saponifiable material is coming into 45 the cleaning bath; elimination of losses by poor guesswork in rule of thumb methods of control and with mixed cleaners where it is necessary to add emulsifier, when it is not needed, because the alkalinity is low.

50     The process will be more readily understood by reference to a specific example. For cleaning steel, an alkali mixture consisting of 55% NaOH, 30% Na<sub>3</sub>PO<sub>4</sub> and 15% Na<sub>2</sub>CO<sub>3</sub> may be employed. Any suitable emulsifier may be used in conjunction with the alkali, as for example, rosin or rosin soap. The alkali mixture and the emulsifier are added to a suitable quantity of water, using about 3½ to 4 ounces of the alkali mixture per gallon of water. The quantity of emulsifier initially introduced is about 10- to 15% by weight of the quantity of alkali. The bath is then ready to be used for cleaning purposes. During the process of cleaning, the concentration of the alkali and of the emulsifier will vary, and these variations 55 may be determined by tests, as outlined, both for

tration by separately adding the alkali or emulsifier or both.

55     For cleaning brass, an alkaline mixture of 50% Na<sub>2</sub>CO<sub>3</sub> 25% Na<sub>3</sub>PO<sub>4</sub> and 25% NaOH may be employed, using initially 5 to 5¼ ounces per gallon of water, and separately adding rosin or other emulsifier in the proportion of 10 to 15% by weight of the alkaline mixture.

60     For cleaning other materials, the composition of the alkaline mixture or emulsifier may be varied according to requirements.

65     My process makes it possible to maintain the solution at its maximum efficiency on varying kinds of work at considerable savings in the amounts of materials used. The process eliminates the necessity of making a large number of mixtures for different classes of work.

70     Where ready-mixed compounds are employed and a slight mistake is made in the quantity of either the emulsifier or the alkali, more of the entire mixture must be used to build up the property necessary. For example, suppose a four ounce concentration gives the right alkalinity, but only one-half the necessary amount of emulsifying power, then it would be necessary to use an eight ounce concentration with consequential waste of material. On the other hand, where four ounces would give the right alkalinity and twice the emulsifying power, in keeping the alkalinity to the correct degree, the solution would soon be saturated because the emulsifiers would carry too great an oil and dirt load. In this case, the whole solution would have to be dumped. 75 These disadvantages are avoided by my process.

75     It will be understood that in the accompanying claims the terms "alkali", "alkaline agent", "emulsifier" and "emulsifying agent" are intended to cover active ingredients of chemical cleaners which are well known in the cleaning art, and which are customarily referred to in the art by these terms, representative ingredients having been set forth in the present specification for the purpose of illustration.

80     What I claim is:

1. A process for continuously maintaining a chemical cleaning solution at maximum operating efficiency, which comprises initially forming an aqueous alkaline solution by admixing predetermined quantities of water, a water-soluble alkaline detergent, and an emulsifying agent capable of reducing the interfacial tension, operating said solution for removing extraneous matter from materials such as metals, clothing, textiles and the like; periodically testing the solution to determine its alkalinity, separately testing the solution for emulsifying power by physically agitating a test portion of the solution with a standard mineral oil and allowing it to separate therefrom, and adjusting the solution by adding the required amount of water-soluble alkaline detergent or water as indicated by the alkalinity test, and the required amount of emulsifying agent or water as indicated by the test for emulsifying power, to restore the solution to its original condition.

85     2. A process for continuously maintaining a chemical cleaning solution at maximum operating efficiency, which comprises initially forming

an aqueous alkaline solution by admixing pre-determined quantities of water, a water-soluble alkaline detergent, and an emulsifying agent capable of reducing the interfacial tension, operating said solution for removing extraneous matter for materials such as metals, clothing, textiles and the like; periodically testing the solution to determine its alkalinity, separately testing the solution for emulsifying power by physically agitating a test portion of the solution with a standard mineral oil and allowing it to separate therefrom, adjusting the solution by adding the re-

quired amount of water-soluble alkaline detergent or water as indicated by the alkalinity test, and the required amount of emulsifying agent or water as indicated by the test for emulsifying power, to restore the solution to its original condition, and periodically permitting said solution to rest to allow excess oil to rise and other extraneous matter removed during the cleaning operation to settle, and removing the said oil and extraneous matter from the solution.

5

10

FRANKLIN H. MACKENZIE.